

Feb. 16, 1926.

W. A. OGG

1,573,015

SMELTING VOLATILIZABLE METALS

Filed May 25, 1925



Inventor:  
William A. Ogg,  
by Emery Booth, James J. James  
Atty.

## UNITED STATES PATENT OFFICE.

WILLIAM A. OGG, OF NEWTON, MASSACHUSETTS.

## SMELTING VOLATILIZABLE METALS.

Application filed May 25, 1925. Serial No. 32,563.

*To all whom it may concern:*

Be it known that I, WILLIAM A. OGG, a citizen of the United States, and a resident of Newton, county of Middlesex, and State of Massachusetts, have invented an Improvement in Smelting Volatilizable Metals, of which the following description, in connection with the accompanying drawings, is a specification, like characters on the drawings 10 representing like parts.

This invention relates to the smelting of material bearing volatilizable metals particularly, but not exclusively, concentrated ores of zinc and has for its object the provision of an efficient and more economical method of smelting as practiced with retorts and condensers. The invention is advantageously but not necessarily practiced in connection with the process more fully described in my prior application, Serial No. 7561, filed Feb. 7, 1925.

My invention will be readily understood by reference to the following description thereof, more particularly when taken in connection with the accompanying drawing illustrating diagrammatically a preferred process exemplifying the invention.

Before proceeding to the description of the process as such, it will be convenient 30 to refer briefly to the furnace commonly used for the reduction of zinc ores or ores of like volatilizable metals. Such a furnace includes tiers of cylindrical retorts as indicated in the diagram by the showing of 35 one such retort at 3, these retorts being commonly made of fire clay or other suitable refractory material and being removable supported in the combustion chamber of the furnace. The ores, which may be 40 metallic oxides or sulphides converted to oxides by roasting, are mixed with the reduction fuel, usually coal or coke free as far as possible from sulphur, and the mixture charged into the retort. In practice, 45 when smelting zinc bearing ores the retorts are subjected to a temperature of about 1300° C. by externally applied heat which reduces the ore and being above the boiling point of zinc volatilizes the metal, which 50 passes out of the retort as a vapor and is condensed to a liquid in a condenser 5, the latter consisting of a short frusto-coni-

cal continuation of the retort projecting from the reduction chamber and being commonly detachably connected with the retort. 55

In conducting the smelting operation it has been common practice to add common salt, sodium chloride, to the charge, for example, a weight of salt equal to about 2% of the weight of the roasted ore. The 60 exact functions of the salt are not exactly understood but it is believed, first, that it acts as a binder on the charge, which is desirable from the operating standpoint; second, that it acts as a flux to make the 65 droplets of zinc in the condenser coalesce; third, that it acts to remove the coating of zinc oxide from the so-called blue powder; and fourth, that it materially reduces the 70 amount of blue powder produced which would require re-smelting.

The introduction of chlorine into the charge by the use of salt produces, of course, a certain amount of zinc chloride which, being volatilizable, is discharged from the 75 retort. In accordance with my present invention I permit a substantial proportion of the vapors to pass from the mouth of the condenser and collect the metal values in these escaping vapors by deposit. Thus, 80 in the diagram I have shown the end of the condenser 5 as entering a hood 7 in which the vapors are preferably burned in a large excess of air to produce a fume product consisting largely of zinc oxide which may be led to a bag house or similar settling chamber, illustrated diagrammatically by the bag 9, wherein the metal values are recovered in the form of a powder or fume. 85 As contrasted with prior processes in which the escape of vapors from the condenser was kept as low as possible and represented a loss, I propose deliberately to operate the furnace so that a substantial fraction of the metal values are passed from the mouth 90 of the condenser and collected as a fume product. On account of the volatility of the zinc chloride it will be substantially entirely carried over in the fume product. Zinc ores also may frequently contain a 95 certain proportion of cadmium and a considerable portion of this metal will be selectively converted to chloride and be carried over into the fume product. Thus, for 100

example, in a case where 2% of salt was utilized in the charge and the fume product collected contained 66.29% metallic zinc, 58.64% was present as zinc oxide and 7.65% as zinc chloride. In the same fume the cadmium content was 1.38%, all of which was present as chloride.

The step of the process just described may preferably be practiced in the manner described in my prior application referred to. Prior to the invention therein described good practice in smelting zinc ore was substantially as follows. The retort was loaded with mixed ore and fuel to roughly 75% of its cubical capacity. The recovery of metal content was about 89½% in the form of spelter and of the remainder about 7.75% was in the residue. About 1% was absorbed by the walls of the retort and the condenser and the remaining loss of 1.75% was principally in the form of escaping vapors from the mouth of the condenser which it was uneconomical to attempt to recover. In accordance with my invention as described in the said application, in order to permit more ore to be treated at one time and to increase the percentage of recovery of metal values minimizing the expense per unit of commercially available metal produced, the retort is deliberately substantially overcharged beyond the capacity of the condenser to condense efficiently and preferably to its full cubical capacity. Sufficient heat is applied to the retorts substantially to reduce all the metal in oxidized form and the condenser is operated at full condensing capacity for the given operating conditions to provide a large recovery of spelter while at the same time by the deliberate overcharge a substantial fraction of the metal values is intentionally caused to escape from the condenser to be recovered by deposit as a fume product.

By utilizing salt in an increased charge of this nature a large recovery of spelter may be provided for with the advantageous functions of salt as utilized in the prior art and the chloride will be collected substantially entirely in the fume product, as will also part of the cadmium value if present.

The presence of chloride in zinc oxide fume is undesirable since zinc chloride is a soluble salt. If only small quantities of chloride were present it would be possible to eliminate them by re-heating but if salt is used and large amounts of metal chloride recovered in the fume as above described, re-heating is not a satisfactory method of purifying the fume. I therefore arrange the separation of the chlorine values from the fume product preferably in such manner as to permit their return to the furnace together with a fresh supply of the roasted zinc ore, or other crude zinc-

bearing material, and reduction fuel to provide a charge for a subsequent volatilizing operation, thus economizing in the use of salt or other fluxing reagent which after the first mix need be added only to make up for operating losses. Furthermore, when the chloride is thus returned to the furnace there is no substantial building up or increase in the relatively undesirable zinc chloride produced as additional amounts of chlorine will not be supplied except as rendered necessary by operating losses.

A preferred method of operation is illustrated diagrammatically in the drawing. The fume product containing zinc oxide and various soluble chlorides may be leached with water, the chlorides appearing in the wash water and an insoluble residue remaining consisting of a very pure zinc oxide unchanged as to the size of particles and which needs only to be dried and disintegrated to restore it to its condition of a very fine zinc oxide free of chloride and other soluble salts and substantially free of lead and cadmium. If the quantity of cadmium in the original ore were substantial, the cadmium may be recovered from the wash water by decanting this wash water to a precipitating tank and adding metallic zinc thereto which will precipitate the cadmium as metal in sponge form, leaving the solution substantially one of pure zinc chloride. This zinc chloride solution may then be treated with a suitable reagent to precipitate the zinc values therefrom and it will be convenient to use an oxide for this purpose, preferably lime, that is, calcium oxide. By the addition of lime zinc hydroxide is precipitated which may readily be converted to the oxide for utilization as such or as a raw material for the production of a high grade of spelter. The calcium chloride solution may then be mixed with further crude zinc-bearing material and reduction fuel to form a charge for a subsequent smelting operation, the calcium chloride taking the place of the salt. The fact that the calcium chloride is recovered in a water solution is not a disadvantage since it is customary and advantageous to wet down the charge of the furnace with water. The calcium chloride solution takes the place of the water as well as of the salt.

The calcium chloride solution is also suitable for use as a binding agent and for this reason may be utilized in connection with reduction fuel and crude zinc-bearing material for the production of briquets, the briquetting of the charge increasing the amount of metal values that may be charged into a retort of given capacity.

I have described in detail one particular

series of operations exemplifying the method of my invention. Obviously these may be widely varied, substituted for by others, added to and in part omitted without departing from the principles of the invention.

What I claim and desire to secure by Letters Patent I shall express in the following claims.

- 10 1. A method of recovering metal values from crude zinc-bearing material which comprises volatilizing the metal content of such material in the presence of chlorine, condensing as metal a major portion of the vapors, collecting an additional portion as a fume product containing the major portion of the chlorine, recovering zinc values from said fume product by treatment with an oxide and mixing the chlorine with fresh 20 crude material and reduction fuel for a subsequent volatilizing operation.

25 2. A method of recovering metal values from crude zinc-bearing material which comprises volatilizing the metal content of such material in the presence of chlorine, condensing as metal a major portion of the vapors, collecting an additional portion as a fume product containing the major portion of the chlorine, leaching the fume product, 30 treating the wash water with an oxide to precipitate the zinc values and mixing the remaining chloride with fresh crude material and reduction fuel for a subsequent volatilizing operation.

35 3. A method of recovering metal values from crude zinc-bearing material which comprises volatilizing the metal content of such material in the presence of chlorine, condensing as metal a major portion of the vapors, collecting an additional portion as a fume product containing the major portion of the chlorine, leaching the fume product, treating the wash water with lime and mixing the resultant solution of calcium chloride 45 with fresh crude material and reduction fuel for a subsequent volatilizing operation.

40 4. A method of recovering metal values from crude zinc-bearing material which comprises volatilizing the metal content of such material in the presence of chlorine, condensing as metal a major portion of the vapors, collecting an additional portion as a fume product containing the major portion of the chlorine and recovering the zinc values 50 occurring as chloride in said fume by treatment with an oxide.

45 5. A method of recovering metal values from crude zinc-bearing material which comprises volatilizing the metal content of such material in the presence of chlorine, condensing as metal a major portion of the vapors, collecting an additional portion as a fume product containing the major portion of the chlorine, leaching the 60 fume, treating the wash water with zinc

to precipitate other metals and recovering the zinc values from the wash water by treatment with an oxide.

6. That method of recovering metal values from crude zinc-bearing materials which comprises volatilizing the metal content of such material in the presence of a fluxing salt, condensing as metal a major portion of the vapors, collecting an additional proportion as a fume product containing the radical of said salt and recovering the zinc values which are combined with said radical by treatment with an oxide.

7. That method of recovering metal values from crude zinc-bearing material utilizing a retort furnace and condenser which comprises charging the retort with a mixture of said material and reduction fuel together with a small quantity of chlorine-bearing material in amount materially in excess of the capacity of the condenser whereby a substantial proportion of the metal values vaporized is discharged in the form of vapor from the condenser mouth, collecting said discharged vapor by deposit as a fume product containing at least a considerable proportion of the chlorine and recovering the zinc values which are combined with chlorine in said fume by treatment with an oxide.

8. That method of recovering metal values from crude zinc-bearing material utilizing a retort furnace and condenser which comprises charging the retort with a mixture of said material and reduction fuel together with a small quantity of chlorine-bearing material in amount materially in excess of the capacity of the condenser whereby a substantial proportion of the metal values vaporized is discharged in the form of vapor from the condenser mouth, collecting said discharged vapor by deposit as a fume product containing at least a considerable proportion of the chlorine, leaching said fume and treating the wash water with an oxide to recover zinc values therefrom.

9. That method of recovering metal values from crude zinc-bearing material utilizing a retort furnace and condenser which comprises charging the retort with a mixture of said material and reduction fuel together with a small quantity of chlorine-bearing material in amount materially in excess of the capacity of the condenser whereby a substantial proportion of the metal values vaporized is discharged in the form of vapor from the condenser mouth, collecting said discharged vapor by deposit as a fume product containing at least a considerable proportion of the chlorine, leaching the fume, precipitating the zinc values from the wash water by a reagent, and mixing the remaining liquid carrying the chlorine with fresh crude material and reduction fuel to provide a charge for a subsequent volatilizing operation.

10. That method of recovering metal values from crude zinc-bearing material utilizing a retort furnace and condenser which comprises charging the retort with a mixture of said material and reduction fuel in amount materially in excess of the capacity of the condenser whereby a substantial proportion of the metal values vaporized is discharged in the form of vapor 5 from the condenser mouth, said mixture also including a quantity of a fluxing compound having a radical forming a soluble salt with zinc, collecting said discharge vapor by deposit as a fume containing at least a considerable proportion of the radical, leaching the fume and precipitating the zinc with a reagent.
11. That method of recovering metal values for crude zinc-bearing material 20 utilizing a retort furnace and condenser which comprises charging the retort with a mixture of said material and reduction fuel in amount materially in excess of the capacity of the condenser whereby a substantial proportion of the metal values vaporized is discharged in the form of vapor from the condenser mouth, said mixture also including a quantity of a fluxing compound having a radical forming a soluble salt with zinc, collecting said discharged vapor by deposit as a fume containing at least a considerable proportion of the radical, leaching the fume, precipitating the zinc with a reagent and mixing the remaining liquid 35 with fresh crude material and reduction fuel to provide a charge for a subsequent volatilizing operation.
12. That method of recovering metal values from crude zinc-bearing material utilizing a retort furnace and condenser 40 which comprises charging the retort with a mixture of said material and reduction fuel in amount materially in excess of the capacity of the condenser whereby a substantial proportion of the metal values vaporized is discharged in the form of vapor from the condenser mouth, said mixture also including a quantity of fluxing haloid, collecting said discharged vapor by deposit as a fume 45 containing a considerable proportion of the halogen, leaching the fume and precipitating the zinc from the wash water.
13. That method of recovering metal values from crude zinc-bearing material utilizing a retort furnace and condenser 55 which comprises charging the retort with a mixture of said material and reduction fuel in amount materially in excess of the capacity of the condenser whereby a substantial proportion of the metal values vaporized is discharged in the form of vapor from the condenser mouth, said mixture also including a quantity of fluxing haloid, collecting said discharged vapor by deposit as a fume 60 containing a considerable proportion of the halogen, leaching the fume, precipitating the zinc from the wash water and mixing the remaining haloid-bearing liquid with fresh crude material and reduction fuel to provide a charge for a subsequent volatilizing 65 operation.

In testimony whereof, I have signed my name to this specification.

WILLIAM A. OGG.